

3,841,982

**METHOD TO IMPROVE THE BRIGHTNESS OF ZINC FROM AN ALKALINE ZINCATE ELECTRODEPOSITION BATH**

Gim Yee, Southfield, Mich., assignor to Oxy Metal Finishing Corporation, Warren, Mich.

No Drawing. Continuation-in-part of application Ser. No. 244,938, Apr. 17, 1972. This application Feb. 20, 1973, Ser. No. 333,927

Int. Cl. C23b 5/10, 5/46

U.S. CL. 204—55 R

36 Claims

**ABSTRACT OF THE DISCLOSURE**

An aqueous alkaline electroplating bath comprising zinc oxide, alkali metal hydroxide, polyethylenimine and a zinc brightening amount of a nitrogen heterocyclic compound of the formula:



wherein X is —S— or



A is independently selected from the group consisting of



n is 0 or 1; when n is 0, nitrogen is doubly bonded to carbon in A; with the proviso that when n is 0, A is



R<sub>1</sub> and R<sub>2</sub> are independently selected from the group consisting of hydrogen, alkyl of 1 to 4 carbon atoms, phenyl; and may be joined to form a six membered aromatic carbocyclic ring and R<sub>3</sub> is hydrogen, alkyl of 1 to 4 carbon atoms or phenyl.

**CROSS REFERENCE TO RELATED CASES**

This case is a continuation-in-part of U.S. Ser. No. 244,938, filed Apr. 17, 1972, now abandoned.

**BACKGROUND OF THE INVENTION**

Zincate plating baths have been used as a means of electrodepositing zinc without employing cyanide ions due to the difficulty in disposing of cyanide ions in waste effluent. Previously, it had been difficult to electrodeposit a bright zinc deposit from a zincate bath over a wide current density area. Some conventional zinc brighteners produce a bright deposit but only over a narrow current density range. The high current density areas generally resulted in a spongy or burnt deposit. It has been found through the combination of brighteners employed in the present case to obtain not only a bright deposit, but also a deposit over a wide current density area.

It has also been found that with conventional brighteners relatively large amounts are required to obtain brightness while with the components of the present invention relatively less amounts are needed to obtain a bright deposit.

Some zinc brighteners have been described in U.S. 3,296,105; U.S. 3,317,412; U.S. 3,393,135; U.S. 3,472,743 and German 1,232,800.

**SUMMARY OF THE INVENTION**

A method is described for obtaining a bright zinc electrodeposit over a wide current density area from a zincate electroplating bath by employing a combination of additives, the first being a polyethylenimine and the second one being a heterocyclic nitrogen containing compound.

**DESCRIPTION OF PREFERRED EMBODIMENTS**

A method is described for obtaining a bright zinc deposit from an alkaline bath preferably a cyanide free alkaline zincate bath wherein the bath contains polyethylenimine and a brightening amount of a nitrogen heterocyclic compound of the structure:



20 wherein X is —S— or



25 A is independently selected from the group consisting of



30 n is 0 or 1; when n is 0, nitrogen is doubly bonded to carbon in A; with the proviso that when n is 0, A is



35 R<sub>1</sub> and R<sub>2</sub> are independently selected from the group consisting of hydrogen, alkyl of 1 to 4 carbon atoms, phenyl; and may be joined to form a six membered aromatic carbocyclic ring and R<sub>3</sub> is hydrogen, alkyl of 1 to 4 carbon atoms or phenyl.

40 Zincate plating baths are those which generally contain zinc oxide and caustic, such as sodium hydroxide. The amount of sodium hydroxide that may be employed ranges from 50 to 250 grams/liter, preferably from about 100 to about 200 grams/liter, while the amount of zinc oxide ranges from 5 to 50 grams/liter, preferably from about 8 to about 30 grams/liter.

45 The processing parameters are such that normally atmospheric temperature and pressure is employed, although temperatures up to 55° C. may also be employed, and even more preferably 15° to about 45° C. The cathode current density ranges from about 5 to 25 amps per sq. ft. while the anode current density ranges from about 10 to 35 amps per sq. ft. where the zinc deposition can occur with agitation.

50 Other agents may also be present in the bath, such as those described in the above patents. Examples of such suitable agents may be anisaldehyde, glue, polyvinyl alcohol and the glycerol ester of polyvinyl alcohol wherein these alcohols have a molecular weight of 5,000 to 20,000. Other polymers that may be employed are gelatin, peptone, and the like. In addition, chelating agents or agents which can form a complex with the metal zinc in the bath may also be employed, such as nitrilotriacetic acid and the various alkali metal salts, such as the sodium salt, ethylenediaminetetraacetic acid, and its water soluble salts, such as sodium, and the like.

55 The polyethylenimine that may be used in the present case has a molecular weight ranging from 1,000 to 400,000, preferably 600 to 60,000 where the percentage of primary, secondary and tertiary nitrogen atoms is about 25, 50, and 25% respectively.

A zincate bath that may be employed in the present invention is as follows:

|                                | Grams/liter |           |
|--------------------------------|-------------|-----------|
|                                | Range       | Preferred |
| Zinc oxide                     | 5-50        | 8-30      |
| NaOH                           | 50-250      | 100-200   |
| Polyethyleneimine              | 0.2-100     | 1-5       |
| Nitrogen heterocyclic compound | 0.005-5     | 0.02-0.08 |
| pH                             | Alkaline    | 10-14     |

The bath pH may be adjusted by adding NaOH.

Some of the nitrogen heterocyclic compounds that may be employed in the present invention are as follows.



wherein  $R_4$  is a "water solubilizing group."

By "water solubilizing group" is meant any substituent on the six membered carbocyclic ring which will improve the water solubility of the compound. Such groups are hydroxy, alkoxy, such as methoxy or ethoxy and the like, carboxy, amino, and the like. In addition,  $R_4$  may be other groups which are not detrimental to the electrodeposition of zinc such as chloro, bromo, cyano ( $-CN$ ), nitro and the like.

#### EXAMPLE 1

A zincate plating bath was formulated containing the following components and was used to electrodeposit zinc onto a steel substrate at a cathode current density of 10 ASF and a temperature of 75° F.

Sodium hydroxide 140 grams/liter; zinc oxide 12 grams/liter; polyethyleneimine (1,200 molecular weight) 2 grams/liter, nitrilotriacetic acid trisodium salt 1 gram/liter; and 2-amino-benzothiazole 0.03 grams/liter.

After plating rod like structures in a typical barrel plating apparatus for 25-30 minutes a uniform bright zinc deposit of 0.2-0.3 mil thickness was obtained. The initial bath pH is about 14.

#### EXAMPLE 2

10 Zincate plating bath similar to the above was also prepared but further including 0.1 g./l. of polyvinyl alcohol. A bright zinc deposit was obtained over a broad current density range following the procedure of Example #1.

#### EXAMPLE 3

15 The procedure of Example #1 was followed, except that the bath also contained 0.1 grams/liter of anisaldehyde with equivalent results being obtained.

#### EXAMPLE 4

20 The procedure of Example #1 was followed, except that the bath also contained 0.1 grams/liter of anisaldehyde and 0.1 grams/liter of polyvinyl alcohol with equivalent results being obtained.

#### EXAMPLE 5

25 A cyanide free alkaline zincate bath was formulated as follows:

|                                              | G./l. |
|----------------------------------------------|-------|
| 30 NaOH -----                                | 140   |
| ZnO -----                                    | 15    |
| 2-mercaptopbenzothiazole -----               | 0.03  |
| polyethyleneimine (1200 molecular wt.) ----- | 3     |

30 Following the procedure of Example #1 equivalently good results were obtained.

What is claimed is:

35 1. An aqueous alkaline electroplating bath comprising inc oxide, alkali metal hydroxide, polyethyleneimine having a molecular weight of from 1,000 to 400,000 and being present in a concentration of 0.2 to 100 grams per liter and a zinc brightening amount of a nitrogen heterocyclic compound of the formula:



40 wherein X is

45  $-S-$  or  $-NR_3$ ; and

49 A is independently selected from the group consisting of

50  $-CN(R_3)_2$ ;  $-C=S$ ;  $-C-S(R_3)$ ;  $-C=NR_3$  and  $-CH$ ;

55 n is 0 or 1; when n is 0, nitrogen is doubly bonded to carbon in A; with the proviso that when n is 0, A is

58  $-CN(R_3)_2$ ;  $-C-S(R_3)$ ; or  $-CH$ ;

60 R<sub>1</sub> and R<sub>2</sub> are independently selected from the group consisting of hydrogen, alkyl of 1 to 4 carbons, phenyl; and may be joined to form a six membered aromatic carbocyclic ring which may be substituted and R<sub>3</sub> is hydrogen, alkyl of 1 to 4 carbon atoms or phenyl.

65 2. The bath of Claim 1 wherein R<sub>1</sub> and R<sub>2</sub> are joined to form a six membered aromatic carbocyclic ring.

70 3. The bath of Claim 2 wherein the carbocyclic ring is substituted by an amino group.

75 4. The bath of Claim 2 wherein the carbocyclic ring is substituted by a bath solubilizing group.

5. The bath of Claim 1 wherein the nitrogen heterocyclic compound is present in an amount ranging from about 0.005 to about 5 grams/liter.

6. The bath of Claim 1 wherein X is  $-S-$ .

7. The bath of Claim 1 wherein X is



8. The bath of Claim 1 wherein A is



9. The bath of Claim 1 wherein A is



10. The bath of Claim 1 wherein A is



11. The bath of Claim 1 wherein A is



12. The bath of Claim 1 wherein n is 0.

13. The bath of Claim 1 wherein R<sub>3</sub> is hydrogen.

14. The bath of Claim 1 wherein R<sub>1</sub> and R<sub>2</sub> are hydrogen.

15. The bath of Claim 1 wherein the nitrogen heterocyclic compound is aminobenzothiazole.

16. The bath of Claim 1 wherein the nitrogen heterocyclic compound is an amino-2-mercaptopbenzothiazole.

17. The bath of Claim 1 wherein the nitrogen heterocyclic compound is 2-imino, 3-alkyl benzothiazole.

18. A method of depositing bright zinc from a zincate electroplating bath comprising electrolyzing the bath of Claim 1 for a period of time sufficient to form a bright zinc deposit onto a cathodic surface.

19. The method of Claim 18 wherein R<sub>1</sub> and R<sub>2</sub> are joined to form a six membered aromatic carbocyclic ring.

20. The method of Claim 19 wherein the carbocyclic ring is substituted by an amino group.

21. The method of Claim 19 wherein the carbocyclic ring is substituted by a bath solubilizing group.

22. The method of Claim 18 wherein the nitrogen heterocyclic compound is present in an amount ranging from about 0.005 to about 5 grams/liter.

23. The method of Claim 18 wherein X is —S—.

24. The method of Claim 18 wherein X is



25. The method of Claim 18 wherein A is



26. The method of Claim 18 wherein A is



27. The method of Claim 18 wherein A is



28. The method of Claim 18 wherein A is



29. The method of Claim 18 wherein n is 0.

30. The method of Claim 18 wherein R<sub>3</sub> is hydrogen.

31. The method of Claim 18 wherein R<sub>1</sub> and R<sub>2</sub> are hydrogen.

32. The method of Claim 18 wherein the nitrogen heterocyclic compound is aminobenzothiazole.

33. The method of Claim 18 wherein the nitrogen heterocyclic compound is an amino-2-mercaptopbenzothiazole.

34. The method of Claim 18 wherein the nitrogen heterocyclic compound is 2-imino, 3-alkyl benzothiazole.

35. The method of Claim 18 wherein the cathodic surface is metallic.

36. A cyanide free alkaline zincate electroplating bath comprising zinc oxide, alkali metal hydroxide, polyethyleneimine having a molecular weight of from 1,000 to 400,000 and being present in a concentration from 0.2 to 100 grams per liter and a zinc brightening amount of a nitrogen heterocyclic compound of the formula:



20 25 wherein X is —S— or



A is independently selected from the group consisting of



n is 0 or 1; when n is 0, nitrogen is doubly bonded to carbon in A; with the proviso that when n is 0, A is



R<sub>1</sub> and R<sub>2</sub> are independently selected from the group consisting of hydrogen, alkyl of 1 to 4 carbon atoms, phenyl; and may be joined to form a six membered aromatic carbocyclic ring which may be substituted and R<sub>3</sub> is hydrogen, alkyl of 1 to 4 carbon atoms or phenyl.

#### References Cited

##### UNITED STATES PATENTS

- |              |        |                              |
|--------------|--------|------------------------------|
| 45 2,853,444 | 9/1958 | Pye et al. ----- 204—55 R X  |
| 2,892,760    | 6/1959 | Gündel et al. ----- 204—44   |
| 3,267,010    | 8/1966 | Creutz et al. ----- 204—52 R |
| 3,672,971    | 6/1972 | Senge et al. ----- 204—55 R  |
| 3,723,263    | 3/1973 | Rosenberg ----- 204—55 R     |

##### FOREIGN PATENTS

- |           |        |                        |
|-----------|--------|------------------------|
| 1,243,488 | 6/1967 | Germany ----- 204—55 R |
| 1,263,445 | 3/1968 | Germany ----- 204—55 R |

50 55 GERALD L. KAPLAN, Primary Examiner